

# UNITED STATES PATENT OFFICE.

ERNEST B. COBB, OF JERSEY CITY, NEW JERSEY, ASSIGNOR TO STANDARD OIL COMPANY (OF NEW JERSEY), OF BAYONNE, NEW JERSEY, A CORPORATION OF NEW JERSEY.

## PROCESS OF PURIFYING HYDROCARBON OILS.

1,387,835.

Specification of Letters Patent. Patented Aug. 16, 1921.

No Drawing.

Application filed April 28, 1920. Serial No. 377,264.

To all whom it may concern:

Be it known that I, ERNEST B. COBB, a citizen of the United States, residing at Jersey City, in the county of Hudson and State of New Jersey, have invented a new and useful Improvement in Processes of Purifying Hydrocarbon Oils, of which the following is a specification.

The present invention relates to the purification or refining of hydro-carbon oils and more particularly to such processes involving the use of strong sulfuric acid, such as acid of 66 degrees Bé. or fuming acid. It is especially applicable in those cases in which the treatment of the oil is heavy, such as in the manufacture of water white lubricating oils, medicinal oils, and the like. It will be fully understood from the following specification, in which it is described in connection with a specific illustration of its use.

A suitable hydro-carbon oil, for example, a petroleum distillate fraction having a gravity heavier than 28° Bé. and a viscosity about 215 at 100° F. (Saybolt) is subjected to successive treatment with about 5 per cent. by volume of 66° Bé., sulfuric acid and with 30—35 per cent. by volume of fuming sulfuric acid (20% anhydrid), the treatment with fuming acid being effected in several dumps, say three or four, with approximately equal proportions of the fuming acid, the oil being cooled between dumps. After the treatment with 66° Bé. acid and after each dump of the fuming acid treatment, the acid sludge may be permitted to settle from the oil and is separated therefrom, carrying with it considerable proportions of the sulfonated compounds produced from the oil. The acid treated oil still contains oil-soluble sulfonated compounds. The oil is then treated in an agitator with about sufficient caustic soda solution of 10 to 16° Bé., or other alkali solution to somewhat more than neutralize the acid, say 10%, allowed to settle, and the spent caustic solution removed. The neutralized oil, which may be blown bright in the agitator, if desired, has a volume about 60% of the original oil treated. The sulfonated compounds of the oil are, by the neutralization process, converted into soaps, which are largely soluble in the oil.

The treated oil containing the oil soluble soaps of the sulfonated compounds is next charged into a still, where it is subjected to

steam distillation until approximately 95% 55 has been distilled off and collected, a temperature below the cracking point of the oil, say 600° F. or thereabouts being maintained. The remaining five per cent. of residue contains substantially all of the sulfo compounds originally present in the oil. The distillate obtained, however, may contain hydrogen sulfid, free sulfur, or compounds which will develop sulfur odors or tastes in the oil. In order to remove these sulfur containing substances from the oil, it may be charged into a still, heated to say 400° F. and treated with steam. It may be steamed for from 2 to 4 hours, after having been heated up, the sulfur and sulfur compounds 60 being thereby eliminated and the viscosity and flash point of the oil brought to the desired figure. The oil may then be steamed until it has a viscosity of 220 to 230 at 100° F. 75

After the treated oil has been steamed, it is again treated with fuming sulfuric acid in less quantity than that used in the first treatment. For example, two dumps of 7½ per cent. of fuming acid each may be 80 utilized, the sludge being separated from the oil after each dump. The effect of this acid treatment is likewise to produce sulfonated compounds, some of which are soluble in the acid and settle out with the sludge, and 85 others remain in the oil. The oil is then slightly over-neutralized by agitation with, say, 5 per cent. by volume of 10—15° Bé. caustic soda solution, the mixture allowed to settle and the spent soda solution drawn off. 90 The oil soluble sulfonated compounds are converted by this process into soap, which remain in solution in the oil. These sulfonated compounds are objectionable, not only for the reason that they tend to produce 95 emulsions when mixed with water, but also for the reason that they interfere seriously with the filtration of the oil, a matter of importance particularly in the case of the production of medicinal oils. After the removal 100 of the spent caustic soda solution, the oil is treated with iso-propyl alcohol, preferably utilizing an aqueous solution containing, for example, 70 per cent. by volume of iso-propyl alcohol having a specific gravity of 105 .81 and 30 per cent. of water. About five per cent. by volume of the iso-propyl alcohol solution is thoroughly agitated with the oil,

2  
and is then allowed to settle. The alcohol solution which settles to the bottom contains the sulfonated compounds, which are removed with it. Some of the alcohol remains 5 in the oil. This may be recovered by heating the oil to 300 to 350 degrees F., thereby vaporizing the alcohol and condensing it, or by blowing the oil with steam at about this temperature. After treatment of the oil in 10 this manner it may be filtered through fullers' earth or a like filtering medium.

Although the present invention has been described in connection with specific details 15 of a particular method of carrying it out, it is not intended that these details shall be regarded as limitations upon the scope 20 of the invention, except in so far as included in the accompanying claims.

I claim:

20 1. The process of treating and purifying hydro-carbon oils which consists in subjecting the oil to the action of strong sulfuric acid, removing oil soluble sulfonated compounds from the treated oils, again treating 25 the oil with strong sulfuric acid and washing the treated oil with iso-propyl alcohol.

2. The process of treating and purifying hydro-carbon oils which consists in subjecting the oil to the action of strong sulfuric 30 acid, removing oil soluble sulfonated compounds from the treated oils, again treating the oil with strong sulfuric acid and washing the treated oil with an aqueous solution of iso-propyl alcohol.

35 3. The process of treating and purifying hydro-carbon oils which consists in subjecting the oil to the action of strong sulfuric

acid, separating and distilling off the greater part of the treated oil, subjecting the distillate to the action of fuming sulfuric acid, and 40 washing the treated oil with an aqueous solution of iso-propyl alcohol.

4. The process of treating and purifying hydro-carbon oils which consists in subjecting a selected fraction thereof to a plurality 45 of treatments with strong sulfuric acid and separating from the oil after each treatment the oil soluble sulfonated derivative produced, the final removal being effected by washing with an aqueous solution of iso- 50 propyl alcohol.

5. The process of treating and refining hydro-carbon oils which consists in subjecting the oil to treatment with fuming sulfuric acid, separating the treated oil and removing therefrom the oil soluble sulfonated 55 derivatives resulting from the acid treatment, again treating the oil with fuming sulfuric acid, neutralizing and washing the treated oil with an aqueous solution of iso-propyl alcohol and steaming the treated oil to remove traces of iso-propyl alcohol therefrom.

6. The process of treating and refining hydro-carbon oils which consists in subjecting said oil to treatment with fuming sulfuric acid, removing the oil soluble sulfonated compounds produced by said treatment from the treated oil, treating said oil to increase its viscosity, again treating the 70 oil with fuming sulfuric acid and washing the retreated oil with an aqueous solution of iso-propyl alcohol.

ERNEST B. COBB.